



US006132911A

# United States Patent [19]

Niimi

[11] Patent Number: 6,132,911

[45] Date of Patent: Oct. 17, 2000

- [54] **METHOD FOR MANUFACTURING PIGMENT, ELECTROPHOTOGRAPHIC PHOTOCONDUCTOR USING THE PIGMENT AND ELECTROPHOTOGRAPHIC IMAGE FORMING METHOD AND APPARATUS USING THE PHOTOCONDUCTOR**
- [75] Inventor: **Tatsuya Niimi**, Numazu, Japan
- [73] Assignee: **Ricoh Company, Ltd.**, Tokyo, Japan
- [21] Appl. No.: **09/359,932**
- [22] Filed: **Jul. 22, 1999**
- [30] **Foreign Application Priority Data**
- Jul. 27, 1998 [JP] Japan ..... 10-225177
- [51] **Int. Cl.<sup>7</sup>** ..... **G03G 5/047**; G03G 13/22; G03G 15/22
- [52] **U.S. Cl.** ..... **430/58.7**; 430/56; 430/59.2; 430/59.4; 430/59.5; 430/78; 430/135; 430/126; 399/159
- [58] **Field of Search** ..... 430/56, 158, 70, 430/59.1, 59.2, 59.4, 59.5, 78, 135, 126

- [56] **References Cited**

## U.S. PATENT DOCUMENTS

- 4,600,674 7/1986 Emoto et al. ..... 430/59.3  
5,395,722 3/1995 Nukada et al. ..... 430/78  
5,418,107 5/1995 Nealey et al. ..... 430/59.5  
5,459,247 10/1995 Hashimoto ..... 430/59.2  
5,874,570 2/1999 Tamura et al. ..... 430/78  
6,026,262 2/2000 Kinoshita et al. ..... 430/56

## FOREIGN PATENT DOCUMENTS

- 60-201352 10/1985 Japan ..... 430/135  
63-237063 10/1985 Japan ..... 430/135

*Primary Examiner*—Roland Martin  
*Attorney, Agent, or Firm*—Cooper & Dunham LLP

- [57]

## ABSTRACT

A method of manufacturing an organic pigment including the steps of providing an organic pigment wet cake which includes at least an organic pigment and a solvent and drying the organic pigment wet cake while the wet cake is heated at a temperature higher than room temperature to prepare a powder of the organic pigment, wherein the organic pigment is present in the organic pigment wet cake in an amount of not greater than about 70% by weight.

**8 Claims, 4 Drawing Sheets**



FIG. 1



FIG. 2



FIG. 3



FIG. 4



FIG. 5



FIG. 6



FIG. 7



FIG. 8



**METHOD FOR MANUFACTURING  
PIGMENT, ELECTROPHOTOGRAPHIC  
PHOTOCOCONDUCTOR USING THE PIGMENT  
AND ELECTROPHOTOGRAPHIC IMAGE  
FORMING METHOD AND APPARATUS  
USING THE PHOTOCOCONDUCTOR**

**BACKGROUND OF THE INVENTION**

**1. Field of the Invention**

The present invention relates to a method for manufacturing organic pigments, an electrophotographic photoconductor using the organic pigments, and an electrophotographic image forming method and apparatus using the electrophotographic photoconductor.

**2. Discussion of the Related Art**

Organic pigments have been used as a filler for paints because a variety of color paints can be prepared by using them, which is an advantage over inorganic pigments. In recent years, attention is focused on organic pigments because of being able to be used as an organic photoelectric conversion material, and therefore various organic pigments have been developed.

When a layer including such an organic pigment is formed, a wet film-forming method is typically used because a layer of large size can be easily formed. As for the wet film-forming method, a method is typically used in which a coating dispersion including an organic pigment is coated on a substrate and dried to form a coating layer on the substrate. The coating properties of the coating layer formed by a wet film-forming method depend on whether the pigment is uniformly dispersed in a vehicle of the coating dispersion during the coating and drying process.

In order to prepare a good coating dispersion in which a pigment is uniformly dispersed, various dispersing devices and systems have been proposed. In addition, various methods for improving dispersion efficiency have also been proposed. When it is desired to prepare a coating dispersion in which pigment particles having a small particle diameter are uniformly dispersed, a dispersing medium (such as balls used for ball milling methods) of small size is typically used. However, even when a small size dispersing medium is used, a good coating dispersion cannot be necessarily prepared if the pigment used has a property such that it is not easily dispersed in the vehicle used. In order to improve the dispersing property of such a coating dispersion, there are two methods in which a large size dispersing medium is used and a pigment which can be easily dispersed is used. When the former method is used, the particle size of the pigment in the resultant dispersion is relatively large compared to that of the pigment in a coating dispersion dispersed by a small size dispersing medium. Therefore, it is preferable to use the latter method. However, it is difficult to design and synthesize a pigment which can be easily dispersed because it is hard to grasp the relationship between the physical and chemical properties of pigment and the dispersing property of the pigment in a coating dispersion.

On the other hand, various information processing systems using electrophotography have been developed in recent years. In particular, photo printers in which information, which is converted to digital signals, is recorded in a photosensitive material using light have been dramatically improved in recording qualities and reliability. This digital recording technique is applied not only for printers, but also for copiers, and so-called digital copiers are developed. Since digital copiers have more information processing functions than analogue copiers, it is supposed

that the demands for digital copiers will increase more and more from now on.

Laser diodes (LDs) and light emitting diodes (LEDs) are typically used as a light source of photo copiers and printers 5 because of being small in size and having good reliability and low manufacturing cost. As for LEDs, an LED emitting light of 660 nm in wavelength is typically used. As for LDs, an LD emitting near infrared light is typically used. Therefore, a need exists for photoconductor having high 10 photosensitivities over a wavelength range of from the visible region to the near-infrared region.

The photosensitivity of an electrophotographic photoconductor almost depends on the photosensitivity of an electron generating material used in the photoconductor. As for 15 charge generating materials, various kinds of materials such as azo type pigments, polycyclic quinone type pigments, trigonal system selenium, phthalocyanine pigments and the like have been developed. Among these pigments, titanyl phthalocyanine (hereinafter referred to as TiOPc) is very 20 useful for a photoconductor for image forming apparatus such as printers and copiers, in which an LED or LD is used as a light source, because of being sensitive to light having a wavelength of from 600 to 800 nm.

In addition, a photoconductor used for electrophotography such as Carson process and the like is required to have 25 the following charge properties as well as the high sensitivity property to the specific light mentioned above:

- (1) a good charging ability in which a high electric potential can be formed and maintained when a photoconductor is 30 charged;
- (2) a good charge decaying ability in which when a photoconductor is exposed to light, the electric potential previously formed on the photoconductor rapidly decays and the residual potential is low; and
- (3) a good charge stability in which a photoconductor can 35 maintain a good charging ability and a good charge decaying ability even when the photoconductor is used for a long time.

In particular, in high sensitive photoconductors such as 40 photoconductors including TiOPc, the charging ability thereof tends to deteriorate and the residual potential tends to increase when the photoconductors are repeatedly used.

Because of these reasons, a need exists for a photoconductor including TiOPc and having a good charge stability. 45

**SUMMARY OF THE INVENTION**

Accordingly, an object of the present invention is to provide 50 a method for preparing an organic pigment which is useful for electrophotographic photoconductor and which is effectively dispersed in a vehicle when a coating dispersion including the pigment is prepared.

Another object of the present invention is to provide a 55 photoconductor which has a high sensitivity and which has good durability such that a good charging ability and charge decaying ability can be maintained even when the photoconductor is repeatedly used for a long time.

Yet another object of the present invention is to provide a 60 coating dispersion useful for manufacturing the photoconductor of the present invention.

A further object of the present invention is to provide an 65 electrophotographic image forming method.

A still further object of the present invention is to provide an 70 electrophotographic image forming process cartridge and apparatus using the photoconductor of the present invention.

To achieve such objects, the present invention contemplates the provision of a method of manufacturing an organic 75

pigment including the steps of preparing an organic pigment wet cake which includes at least an organic pigment and a solvent, and drying the organic pigment wet cake by heating the wet cake at a temperature higher than room temperature to prepare a powder of the organic pigment, wherein the organic pigment is present in the organic pigment wet cake in an amount of not greater than about 70% by weight at the beginning of the drying step.

Preferably, the content of the pigment in the wet cake is not greater than about 50% by weight.

In addition, the heating step is preferably performed under a reduced atmospheric pressure not greater than 10 mm Hg.

Further, the organic pigment is a phthalocyanine pigment, and more specifically is a titanyl phthalocyanine compound which has an X-ray diffraction spectrum such that a maximum diffraction peak is observed at an Bragg (2  $\theta$ ) angle of  $27.2\pm0.2^\circ$  when a specific X-ray of Cu—K  $\alpha$  (wavelength of 1.514 Å) irradiates the titanyl phthalocyanine compound.

In another aspect of the present invention, a coating dispersion useful for manufacturing an electrophotographic photoconductor is provided in which the organic pigment prepared by the method of the present invention mentioned above is dispersed in a solvent.

In yet another aspect of the present invention, an electrophotographic photoconductor is provided which has a photoconductive layer formed overlying an electroconductive substrate and including the organic pigment prepared by the method of the present invention mentioned above.

In a further aspect of the present invention, an electrophotographic image forming apparatus is provided which includes the photoconductor of the present invention mentioned above.

These and other objects, features and advantages of the present invention will become apparent upon consideration of the following description of the preferred embodiments of the present invention taken in conjunction with the accompanying drawings.

#### BRIEF DESCRIPTION OF THE DRAWINGS

FIG. 1 is a schematic diagram illustrating a sectional view of an embodiment of the electrophotographic photoconductor of the present invention;

FIG. 2 is a schematic diagram illustrating a sectional view of another embodiment of the electrophotographic photoconductor of the present invention;

FIG. 3 is a schematic diagram illustrating a sectional view of yet another embodiment of the electrophotographic photoconductor of the present invention;

FIG. 4 is a schematic diagram illustrating a main part of an embodiment of the electrophotographic image forming apparatus of the present invention;

FIG. 5 is a schematic diagram illustrating a main part of another embodiment of the electrophotographic image forming apparatus of the present invention;

FIG. 6 is a schematic diagram illustrating an embodiment of the electrophotographic image forming process cartridge of the present invention;

FIG. 7 is a graph illustrating the X-ray diffraction spectrum of an embodiment of the titanyl phthalocyanine pigment prepared by the method of the present invention; and

FIG. 8 is a graph illustrating the X-ray diffraction spectrum of an embodiment of the titanyl phthalocyanine pigment prepared by a comparative method.

#### DESCRIPTION OF THE PREFERRED EMBODIMENTS

The dispersing properties of an organic pigment in a dispersion is broadly classified into a property to be pulver-

ized (pulverizability) and dispersion stability. The dispersion stability of a dispersion including a pigment and a vehicle mainly depends on the factors such as wettability of the pigment with the vehicle, the particle size of the pigment, and the difference between the specific gravities of the pigment and the vehicle. The pulverizability mainly depends on the hardness of a pigment when pulverizing conditions are constant. A hard organic pigment generally has a high bulk density.

Bulk density of organic pigments depends on not only their true specific gravity, but also their cohesive force. Although the minimum unit of organic pigment particles is a primary particle, the primary particle typically aggregates by an interaction between the primary particles such as intermolecular hydrogen bonding, resulting in formation of secondary particles. The particle size of primary particles of a pigment is determined depending on the synthesis conditions of the pigment unless a method such as an acid pasting method in which the pigment is solved is used. On the other hand, the particle size of secondary particles varies depending on the conditions of processes performed after the synthesis process. The greater the particle size of the secondary particles of a pigment, i.e., the more the primary particles of a pigment aggregate, the higher the bulk density of the pigment.

As mentioned above, organic pigments are used as a photoelectric converting material in recent years. In general, an organic pigment having a good photoelectric converting property tends to have a strong cohesive force, and therefore the organic pigment tends to have a high bulk density. Accordingly, it is difficult to uniformly disperse such an organic pigment having a good photoelectric converting property in order to prepare a good coating dispersion. In addition, there is a case that among organic pigments having the same chemical structure, only an organic pigment having a specified crystal form has a good photoelectric converting property. The crystal form of a pigment easily changes by mechanical and physical stresses applied to the pigment during a pulverizing process as well as chemical stresses, and therefore it is not preferable to prepare a coating dispersion while applying too much stresses. Therefore, a need exists for an organic pigment which has a good photoelectric converting property and which can be easily dispersed.

The present invention is to provide a method of manufacturing an organic pigment having a good dispersing property. The method is characterized in that a powder of an organic pigment can be prepared by decreasing aggregation of the primary particles of the pigment while the particle size of the primary particles and the crystal form of the pigment are maintained. The thus prepared organic pigment can be easily dispersed in a vehicle, and thereby a good coating dispersion, which is useful for forming a photoconductive layer, can be prepared.

In the present invention, a method for manufacturing an organic pigment is provided which includes the steps of preparing an organic pigment wet cake which includes at least an organic pigment and a solvent, and drying the organic pigment wet cake by heating the wet cake at a temperature higher than room temperature to prepare a powder of the organic pigment, wherein the organic pigment is present in the organic pigment wet cake in an amount of not greater than about 70% by weight at the beginning of the drying step.

Hereinafter the present invention will be described in detail. Organic pigments are generally manufactured by a wet process. For example, the wet process is performed as follows:

- (1) a pigment is synthesized in a solvent;
- (2) the synthesized pigment is washed with a solvent;
- (3) the pigment is refined by, for example, recrystallization; and
- (4) the crystal form of the refined pigment is changed, if desired.

These operations are performed while the pigment is dispersed in a liquid. The thus prepared dispersion including a pigment is filtered or centrifuged to prepare a wet cake of the pigment, and then the wet cake is dried to prepare a powder of the pigment.

If the wet cake has a solid content not less than about 70% by weight when the wet cake is prepared by filtering or centrifuging, a pigment powder having a high bulk density is prepared. As mentioned above, a pigment powder having a high bulk density cannot easily pulverized, i.e., the pulverizing efficiency is low. Therefore, a high mechanical or physical stress is needed to pulverize the pigment, resulting in occurrence of a problem such as change of its crystal form.

When a wet cake having a solid content not greater than about 70% by weight is rapidly dried at a temperature higher than room temperature, a powder having a low bulk density can be formed. This is because the wet cake having a solid content not greater than about 70% by weight includes a considerable amount of a solvent and therefore has a low bulk density itself. To perform the drying operation under a reduced pressure not greater than 10 mm Hg brings better results. The solid content of a pigment in a wet cake is preferably not greater than about 50% by weight. When the solid content is too low, a problem which occurs is that it is not easy to handle the wet cake and it takes a long time to dry the wet cake, resulting in increase of manufacturing cost. Therefore the solid content is preferably from about 20% to about 70%.

Organic pigments for use in the present invention include known organic pigments. Specific examples of such pigments include phthalocyanine type pigments, monoazo pigments, disazo pigments, trisazo pigments, perylene type pigments, perynone type pigments, quinacridone type pigments, quinone type condensation polycyclic compounds, squaric acid type dyes, naphthalocyanine type pigments, azulениum salt type dyes and the like.

Among these pigments, phthalocyanine type pigments are preferable because of having a variety of crystal forms. Of these phthalocyanine pigments, titanyl phthalocyanine has a property such that its carrier generating ability dramatically changes depending on the crystal forms. In particular, titanyl phthalocyanine, which has an X-ray spectrum such that a maximum diffraction peak is observed at a Bragg (2θ) angle of  $27.2^\circ \pm 0.2^\circ$  when a specific X-ray of Cu—K α having a wavelength of 1.514 Å irradiates the pigment, has a very high photo-carrier generating ability. However, the pigment is unstable and therefore easily changes to another crystal form. According to the present invention, a dispersion in which titanyl phthalocyanine having a desired crystal form is dispersed can be stably prepared.

As for the dryers for drying wet cakes of pigments by heating to a temperature higher than room temperature, known dryers can be used. When the drying operation is performed in the atmosphere, an air blowing type dryer is preferable. In addition, it is preferable to perform the drying operation under a reduced atmospheric pressure if a pigment to be dried easily decomposes or changes its crystal form at a high temperature. The pressure of the reduced atmospheric pressure is preferably not greater than 10 mm Hg (i.e., a higher vacuum state than a state in which the atmospheric pressure is 10 mm Hg).

Next, coating dispersions of the present invention useful for preparing electrophotographic photoconductors will be explained. When a coating dispersion including a pigment useful for an electrophotographic photoconductor are prepared, the pigment has to be dispersed while maintaining its crystal form if desired functions of the photoconductor can be obtained only by the pigment having the crystal form. In recent years, resolution of reproduced images is regarded as the most important property in electrophotography, and therefore the particle diameter of a pigment included in a photoconductor becomes smaller and smaller. When a dispersion including a small size pigment is prepared, it is important to use a pigment which has a small particle diameter and which is easily dispersed in a vehicle used. By using the pigment having a low bulk density prepared by the method of the present invention, such a desired dispersion can be prepared.

The coating dispersion of the present invention can be prepared by any known method. For example, a pigment is dispersed in a proper solvent, if desired, together with a binder resin using a dispersing device such as ball mills, attritors, sand mills and super sonic dispersing machines. As for the binder resin, one or more binder resins are selected from known resins such that the resultant photoconductor has desired charge properties. In addition, the solvent is also selected from known solvents such that the pigment used is easily wet with the solvent and is stably dispersed therein. The solvent may be different from or the same as the solvent included in the wet cake.

Hereinafter, the electrophotographic photoconductor of the present invention will be explained referring to figures.

FIG. 1 is a schematic view illustrating a cross section of an embodiment of the electrophotographic photoconductor of the present invention. In FIG. 1, a single-layer type photoconductive layer 33 which is mainly constituted of a charge generating material and a charge transporting material is formed on an electroconductive substrate 31.

FIGS. 2 and 3 are schematic views illustrating cross sections of other embodiments of the electrophotographic photoconductor of the present invention. The photoconductors as shown in FIGS. 2 and 3 have multi-layer structures in which a charge generating layer 35 which is mainly constituted of a charge generating material and a charge transporting layer 37 which is mainly constituted of a charge transporting material are overlaid.

Suitable materials for use as the electroconductive substrate include materials having a volume resistance not greater than  $10^{10} \Omega \text{ cm}$ . Specific examples of such materials include plastic cylinders, plastic films or paper sheets, on the surface of which a metal such as aluminum, nickel, chromium, nichrome, copper, gold, silver, platinum and the like, or a metal oxide such as tin oxides, indium oxides and the like, is deposited or sputtered. In addition, a tube can also be used as the substrate 31 which is prepared by tubing a plate of a metal such as aluminum, aluminum alloys, nickel, stainless steel and the like or tubing by a method such as impact ironing or direct ironing, and then treating the surface of the tube by cutting, super finishing, polishing and the like. Further, endless belts of a metal such as nickel, stainless steel and the like, which have been disclosed, for example, in Japanese Laid-Open Patent Publication No. 52-36016, can also be used as the substrate 31.

Furthermore, substrates, in which a coating liquid including a binder resin and an electroconductive powder is coated on the supporters mentioned above, can be used as the substrate 31. Specific examples of the electroconductive powder include carbon black, acetylene black, powders of

metals such as aluminum, nickel, iron, nichrome, copper, zinc, silver and the like, and metal oxides such as electroconductive tin oxides, ITO and the like. Specific examples of the binder resin include known thermoplastic resins, thermosetting resins and photo-crosslinking resins, such as polystyrene, styrene-acrylonitrile copolymers, styrene-butadiene copolymers, styrene-maleic anhydride copolymers, polyesters, polyvinyl chloride, vinyl chloride-vinyl acetate copolymers, polyvinyl acetate, polyvinylidene chloride, polyarylates, phenoxy resins, polycarbonates, cellulose acetate resins, ethyl cellulose resins, polyvinyl butyral resins, polyvinyl formal resins, polyvinyl toluene, poly-N-vinyl carbazole, acrylic resins, silicone resins, epoxy resins, melamine resins, urethane resins, phenolic resins, alkyd resins and the like. The electroconductive layer can be formed by coating a coating liquid in which an electroconductive powder and a binder resin are dispersed or dissolved in a proper solvent such as tetrahydrofuran, dichloromethane, methyl ethyl ketone, toluene and the like, and then drying the coated liquid.

In addition, substrates, in which an electroconductive resin film is formed on a surface of a cylindrical substrate using a heat-shrinkable resin tube which is made of a combination of a resin such as polyvinyl chloride, polypropylene, polyesters, polyvinylidene chloride, polyethylene, chlorinated rubber and fluorine-containing resins, with an electroconductive material, are also used as the substrate 31.

Next, the photoconductive layer of the photoconductor of the present invention will be explained.

In the present invention, the photoconductive layer may be a single-layer type photoconductor or a multi-layer type photoconductor.

At first, multi-layer type photoconductors in which the charge generating layer 35 and the charge transporting layer 37 are overlaid will be explained.

In the charge generating layer 35, an organic pigment which is prepared by the aforementioned method of the present invention is mainly included as the charge generating material. The organic pigment is dispersed in a proper solvent, if desired together with a binder resin, using a dispersing device such as ball mills, attritors, sand mills and super sonic dispersing machines to prepare a coating liquid. The thus prepared coating liquid is coated on a substrate 31 and dried, resulting in formation of the charge generating layer 35.

Suitable binder resins, which are optionally mixed in the charge generating layer coating liquid, include polyamides, polyurethanes, epoxy resins, polyketones, polycarbonates, silicone resins, acrylic resins, polyvinyl butyral, polyvinyl formal, polyvinyl ketones, polystyrene, polysulfone, poly-N-vinylcarbazole, polyacrylamide, polyvinyl benzal, polyesters, phenoxy resins, vinyl chloride-vinyl acetate copolymers, polyvinyl acetate, polyphenylene oxide, polyamides, polyvinyl pyridine, cellulose resins, casein, polyvinyl alcohol, polyvinyl pyrrolidone, and the like. The content of the binder resin in the charge generating layer 35 is preferably from 0 to 500 parts by weight, and more preferably from 0 to 300 parts by weight, per 100 parts by weight of a charge generating material.

Suitable solvents for use in the charge generating layer coating liquid include isopropanol, acetone, methyl ethyl ketone, cyclohexanone, tetrahydrofuran, dioxane, ethyl cellosolve, ethyl acetate, methyl acetate, dichloromethane, monochlorobenzene, cyclohexane, toluene, xylene, ligroin, and the like.

The coating liquid can be coated by a coating method such as dip coating, spray coating, bead coating, nozzle coating, spinner coating and ring coating. The thickness of the charge generating layer 35 is preferably from 0.01 to 5  $\mu\text{m}$ , and more preferably from 0.1 to 2  $\mu\text{m}$ .

The charge transporting layer **37** can be formed by coating a charge transporting layer coating liquid, which is prepared by dispersing or dissolving a charge transporting material and a binder resin in a proper solvent, on the charge generating layer **35**, and then drying the coated liquid. In addition, additives such as a plasticizer, a leveling agent, an antioxidant and the like can be added in the coating liquid, if desired.

Charge transporting materials are classified into positive-hole transporting materials and electron transporting materials.

Specific examples of the electron transporting materials include electron accepting materials such as chloranil, bromanil, tetracyanoethylene, tetracyanoquinodimethane, 2,4,7-trinitro-9-fluorenol, 2,4,5,7-tetranitro-9-fluorenol, 2,4,5,7-tetranitroxanthone, 2,4,8-trinitrothioxanthone, 2,6,8-trinitro-4H-indeno[1,2-b]thiophene-4-one, 1,3,7-trinitro dibenzothiophene-5,5-dioxide, benzoquinone derivatives and the like.

Specific examples of the positive-hole transporting materials include known materials such as poly-N-carbazole and its derivatives, poly- $\gamma$ -carbazoleylethylglutamate and its derivatives, pyrene-formaldehyde condensation products and their derivatives, polyvinyl pyrene, polyvinyl phenanthrene, polysilane, oxazole derivatives, oxadiazole derivatives, imidazole derivatives, monoarylamines, diarylamines, triarylamines, stilbene derivatives,  $\alpha$ -phenyl stilbene derivatives, benzidine derivatives, diarylmethane derivatives, triaryl methane derivatives, 9-styrylanthracene derivatives, pyrazoline derivatives, divinyl benzene derivatives, hydrazone derivatives, indene derivatives, butadiene derivatives, pyrene derivatives, bisstilbene derivatives, enamine derivatives, and the like.

These charge transporting materials are used alone or in combination.

Suitable binder resins for use in the charge transporting layer coating liquid include thermoplastic or thermosetting resins such as polystyrene, styrene-acrylonitrile copolymers, styrene-butadiene copolymers, styrene-maleic anhydride copolymers, polyesters, polyvinyl chloride, vinyl chloride-vinyl acetate copolymers, polyvinyl acetate, polyvinylidene chloride, polyarylates, phenoxy resins, polycarbonates, cellulose acetate resins, ethyl cellulose resins, polyvinyl butyral resins, polyvinyl formal resins, polyvinyl toluene, poly-N-vinyl carbazole, acrylic resins, silicone resins, epoxy resins, melamine resins, urethane resins, phenolic resins, alkyd resins and the like.

The content of the charge transporting material in the charge transporting layer 37 is preferably from 20 to 300 parts by weight, and more preferably from 40 to 150 parts by weight, per 100 parts by weight of the binder resin. The thickness of the charge transporting layer 37 is preferably from about 5 to 100  $\mu\text{m}$ .

Suitable solvent for use in the charge transporting layer coating liquid include tetrahydrofuran, dioxane, toluene, dichloromethane, monochlorobenzene, dichloroethane, cyclohexanone, methyl ethyl ketone, acetone and the like.

In the charge transporting layer 37, a high molecular weight charge transporting material, which serves as a charge transporting material and a binder resin, can be preferably used. When the charge transporting layer 37 is constituted of a high molecular weight charge transporting material, the charge transporting layer 37 has good abrasion resistance. Suitable high molecular weight charge transporting materials for use in the charge transporting layer 37 include known high molecular weight charge transporting materials. Among these materials, polycarbonates having a triarylamine structure in the main chain and/or the side chain thereof are preferably used. In particular, the materials represented by the following formulas (1) to (10) are more preferably used.



wherein R1, R2 and R3 independently represent an alkyl group which is substituted or is not substituted, or a halogen atom; R4 represents a hydrogen atom, or an alkyl group which is substituted or is not substituted; R5, and R6 independently represent an aryl group which is substituted or is not substituted; r, p and q independently represent 0 or an integer of from 1 to 4; k is a number of from 0.1 to 1.0 and j is a number of from 0 to 0.9; and n is an integer of from 5 to 5000; and X represents a divalent aliphatic group, a divalent alicyclic group or a divalent group having the following formula:



wherein R101 and R102 independently represent an alkyl group which is substituted or is not substituted, an aryl group which is substituted or is not substituted, or a halogen atom; t and m represent 0 or an integer of from 1 to 4; v is 0 or 1; and Y represents a linear alkylene group, a branched alkylene group, a cyclic alkylene group, —O—, —S—, —SO—, —SO<sub>2</sub>—, —CO—, —CO—O—Z—O—CO— (Z represents a divalent aliphatic group), or a group having the following formula:



wherein a is an integer of from 1 to 20; b is an integer of from 1 to 2000; and R103 and R104 independently represent an alkyl group which is substituted or is not substituted, or an aryl group which is substituted or is not substituted, wherein R101, R102, R103 and R104 may be the same or different from each other.

(1)



wherein R7 and R8 independently represent an aryl group which is substituted or is not substituted; Ar1, Ar2 and Ar3 independently represent an aryl group; and X, k, j and n are defined above in formula (1).



wherein R9 and R10 independently represent an aryl group which is substituted or is not substituted; Ar4, Ar5 and Ar6 independently represent an aryl group; and X, k, j and n are defined above in formula (1).

(4)



wherein R11 and R12 independently represent an aryl group which is substituted or is not substituted; Ar7, Ar8 and Ar9 independently represent an aryl group; p is an integer of from 1 to 5; and X, k, j and n are defined above in formula (1).



wherein R13 and R14 independently represent an aryl group which is substituted or is not substituted; Ar10, Ar11 and Ar12 independently represent an arylene group; X1 and X2 independently represent an ethylene group which is substituted or is not substituted, or a vinylene group which is substituted or is not substituted; and X, k, j and n are defined above in formula (1).

15 group which is substituted or is not substituted, a cycloalkylene group which is substituted or is not substituted, an alkyleneether group which is substituted or is not substituted, an oxygen atom, a sulfur atom, or a vinylene group; u, v and w independently represent 0 or 1; and X, k, j and n are defined above in formula (1).



wherein R15, R16, R17 and R18 independently represent an aryl group which is substituted or is not substituted; Ar13, Ar14, Ar15 and Ar16 independently represent an arylene group; Y1, Y2 and Y3 independently represent an alkylene group; Y1, Y2 and Y3 independently represent an alkylene

20 group which is substituted or is not substituted, a cycloalkylene group which is substituted or is not substituted, an alkyleneether group which is substituted or is not substituted, an oxygen atom, a sulfur atom, or a vinylene group; u, v and w independently represent 0 or 1; and X, k, j and n are defined above in formula (1).

35

wherein R19 and R20 independently represent a hydrogen atom, or aryl group which is substituted or is not substituted, and R19 and R20 may form a ring; Ar17, Ar18 and Ar19 independently represent an arylene group; and X, k, j and n are defined above in formula (1).

(7)



50

wherein R21 represents an aryl group which is substituted or is not substituted; Ar20, Ar21, Ar22 and Ar23 independently represent an arylene group; and X, k, j and n are defined above in formula (1).



wherein R22, R23, R24 and R25 independently represent an aryl group which is substituted or is not substituted; Ar24, Ar25, Ar26, Ar27 and Ar28 independently represent an arylene group; and X, k, j and n are defined above in formula (1).

As for the binder resin for use in the photoconductive layer 33, the resins mentioned above for use in the charge transporting layer 37 can be used. In addition, the resins mentioned above for use in the charge generating layer 35



wherein R26 and R27 independently represent an aryl group which is substituted or is not substituted; Ar29, Ar30 and Ar31 independently represent an arylene group; and X, k, j and n are defined above in formula (1).

The charge transporting layer 37 may include an additive such as plasticizers and leveling agents. Specific examples of the plasticizers include dibutyl phthalate, diethyl phthalate and the like, which are used as the plasticizer for resins. The content of the plasticizer in the charge transporting layer 37 is preferably from 0 to about 30 parts by weight per 100 parts by weight of the binder resin. Specific examples of the leveling agent include silicone oils such as dimethylsilicone oil, and methylphenylsilicone oil, and polymers or oligomers which have a perfluoroalkyl group in their side chain. The content of the leveling agent in the charge transporting layer 37 is preferably from 0 to about 1 part by weight per 100 parts by weight of the binder resin.

Next, a single-layer type photoconductor will be explained. In the single-layer type photoconductor, the organic pigment prepared by the aforementioned method of the present invention can also be used. The photoconductive layer 33 can be formed on the substrate 31 by coating a coating liquid, which is prepared by dispersing or dissolving a charge generating material and a binder resin in a proper solvent, and then drying the coated liquid. In the photoconductive layer 33, one or more of the charge transporting materials (1) to (10) mentioned above can be added to prepare a functionally separated photoconductor. In addition, an additive such as plasticizers, leveling agents and antioxidants may be included.

can also be used. Needless to say, the high molecular weight charge transporting materials can be preferably used. The content of the charge generating material in the photoconductive layer 33 is preferably from 5 to 40 parts by weight per 100 parts by weight of the binder resin included in the

photoconductive layer 33. The content of the charge transporting material in the photoconductive layer 33 is preferably from 0 to 190 parts by weight, and more preferably from 50 to 150 parts by weight, per 100 parts by weight of the binder resin included in the photoconductive layer 33. The photoconductive layer 33 can be formed by coating a coating liquid which is prepared by dispersing a charge generating material and a binder resin, if desired together with a charge transporting material, in a proper solvent such as tetrahydrofuran, dioxane, dichloroethane, cyclohexane and the like using a dispersing device, and drying the coated liquid. Suitable coating methods include dip coating, spray coating, bead coating and the like. The thickness of the photoconductive layer 33 is preferably from 5 to 100  $\mu\text{m}$ .

The photoconductors of the present invention may include an undercoat layer between the electroconductive substrate 31 and the photoconductive layer. The undercoat layer mainly includes a resin. Since a photoconductive layer is typically formed on the undercoat layer by coating a liquid including an organic solvent, the resin in the undercoat layer preferably has good resistance to the organic solvent. Specific examples of such resins include water-soluble resins such as polyvinyl alcohol resins, casein and polyacrylic acid sodium salts; alcohol soluble resins such as nylon copolymers and methoxymethylated nylon resins; and thermosetting resins capable of forming a three-dimensional network such as polyurethane resins, melamine resins, alkyd-melamine resins, epoxy resins and the like.

The undercoat layer may include a fine powder of metal oxides such as titanium oxide, silica, alumina, zirconium

## 15

oxide, tin oxide and indium oxide to prevent the occurrence of moire of the resultant recorded images and to decrease residual surface potential of the photoconductor. The under-coat layer can also be formed by coating a coating liquid using a proper solvent and a proper coating method as mentioned above in the photoconductive layer.

A metal oxide layer which is formed, for example, by a sol-gel method using a silane coupling agent, titanium coupling agent or a chromium coupling agent can also be used as an undercoat layer.

A layer of aluminum oxide which is formed by an anodic oxidation method and a layer of an organic compound such as polyparaxylylene or an inorganic compound such as SiO<sub>2</sub>, SnO<sub>2</sub>, TiO<sub>2</sub>, ITO or CeO<sub>2</sub> which is formed by a vacuum evaporation method are also preferably used as an undercoat layer. The thickness of the under-coat layer is preferably 0 to about 5  $\mu\text{m}$ .

The photoconductors of the present invention may include a protective layer, which is formed overlying the photoconductive layer, to protect the photoconductive layer. Suitable materials for use in the protective layer include ABS resins, ACS resins, olefin-vinyl monomer copolymers, chlorinated polyethers, aryl resins, phenolic resins, polyacetal, polyamides, polyamideimide, polyacrylates, polyarylsulfone, polybutylene, polybutylene terephthalate, polycarbonate, polyethersulfone, polyethylene, polyethylene terephthalate, polyimides, acrylic resins, polymethylpentene, polypropylene, polyphenyleneoxide, polysulfone, polystyrene, AS resins, butadiene-styrene copolymers, polyurethane, polyvinyl chloride, polyvinylidene chloride, epoxy resins and the like. The protective layer may include a fluorine-containing resin or a silicone resin to improve abrasion resistance of the photoconductor. The protective layer may include an inorganic filler such as titanium oxide, tin oxide, potassium titanate and the like, which is dispersed in a resin.

The protective layer can be formed by a conventional coating method. The thickness of the protective layer is from 0.1 to 10  $\mu\text{m}$ . In addition, a layer of amorphous carbon or amorphous silicon carbide which is formed by a vacuum evaporation method can also be used as the protective layer.

In the present invention, an intermediate layer may be formed between the photoconductive layer and the protective layer. The intermediate layer is mainly constituted of a resin. Specific examples of the resin include polyamides, alcohol soluble nylons, polyvinyl butyral having a hydroxide group, polyvinyl butyral, polyvinyl alcohol, and the like. The intermediate layer can be formed by the above-mentioned conventional coating method. The thickness of the intermediate layer is preferably from 0.05 to 2  $\mu\text{m}$ .

Hereinafter the image forming method and image forming apparatus using the photoconductor of the present invention will be explained referring to figures.

FIG. 4 is a schematic view illustrating a main part of an embodiment of the image forming apparatus of the present invention.

In FIG. 4, numeral 1 denotes a cylindrical photoconductor. The photoconductor 1 has a photoconductive layer in which a pigment prepared by the method of the present invention is included. Around the photoconductor 1, a discharging lamp 2, a charger 3, an eraser 4, a light image irradiating device 5, a developing unit 6, a pre-transfer charger 7, a transfer charger 10, a separating charger 11, a separating pick 12, a pre-cleaning charger 13, a fur brush 14, and a cleaning brush 15 are counterclockwise configured in this order. In addition, a pair of registration rollers 8 are provided to feed a transfer paper 9 to the space between the

## 16

photoconductor 1 and the transfer charger 10 (and the separating charger 11). The photoconductor 1, which is constituted of an electroconductive substrate and a photoconductive layer formed on the substrate, rotates in a direction indicated by an arrow.

The photoconductor 1 is positively or negatively charged with the charger 3 while the photoconductor is rotating. Residual toner is removed from the photoconductor 1 by the eraser 4, and then the light image irradiating device 5 irradiates the photoconductor 1 with imagewise light to form an electrostatic latent image on the photoconductor 1.

A conventional transfer charger can be used as the transfer device of the image forming apparatus of the present invention; however, the above-mentioned transfer device, i.e., a combination of the transfer charger 10 with the separating charger 11, is preferable.

Suitable light sources for use in the light image irradiating device 5 and the discharging lamp 2 include fluorescent lamps, tungsten lamps, halogen lamps, mercury lamps, sodium lamps, light emitting diodes (LEDs), laser diodes (LDs), light sources using electroluminescence (EL), and the like. In addition, in order to obtain light having a desired wave length range, filters such as sharp-cut filters, band pass filters, near-infrared cutting filters, dichroic filters, interference filters, color temperature converting filters and the like can be used. These light sources can also be used for the image transfer process, discharging process, and cleaning process, and a pre-exposure process which is optionally performed, if it is needed to irradiate light to the photoconductor 1 in the processes.

The electrostatic latent image formed on the photoconductor 1 is then developed with a toner on a developing roller 61 in the developing unit 6. The toner image formed on the photoconductor 1 is then charged with the pre-transfer charger 7 so that the toner image has a charge suitable for transferring. The toner image is then transferred onto the transfer paper 9 while the transfer paper 9 is charged with the transfer charger 10. The transfer paper 9 is then charged with the separating charger 11 so as to easily separate from the photoconductor 1 by being released from the state in which the transfer paper 9 and the photoconductor 1 are adhered to each other electrostatically. The transfer paper 9 is then separated from the photoconductor 1 with the separating pick 12. After the toner image transferring process, the surface of the photoconductor 1 is cleaned using the pre-cleaning charger 13, the fur brush 14 and the cleaning brush 15. The residual toner remaining on the photoconductor 1 can be removed by only the cleaning brush 15.

When imagewise light irradiates the photoconductor 1 which is previously charged positively or negatively, an electrostatic latent image having a positive or negative charge is formed on the photoconductor 1. When the latent image having a positive (negative) charge is developed with a toner having a negative (positive) charge, a positive image (i.e., the same image as the latent image) can be obtained. In contrast, when the latent image having a positive (negative) charge is developed with a toner having a positive (negative) charge, a negative image (i.e., a reversal image) can be obtained. As for the developing method, a conventional developing method can be used. In addition, as for the discharging method, a conventional method can also be used.

In this embodiment of the image forming apparatus, a cylindrical photoconductor is used; however, a sheet-shaped or endless-belt-shaped photoconductor can also be used. In addition, corotrons, scorotrons, solid state chargers, and charging rollers can be used as the pre-cleaning charger 13.

These chargers can also be used as a substitute for the transfer charger **10** and the separating charger **11**; however, the unity of the transfer charger **10** and the separating charger **11** is preferable because of being efficient. Further, known brushes such as fur brushes and magnetic fur brushes can be used as the cleaning brush **15**.

FIG. 5 is a schematic view illustrating a main part of another embodiment of the image forming apparatus of the present invention. In this embodiment, a belt-shaped photoconductor **21** is used. The photoconductor **21** has a photoconductive layer including an organic pigment prepared by the method of the present invention. The belt-shaped photoconductor **21** is rotated by rollers **22a** and **22b**. The photoconductor **21** is charged with a charger **23**, and then light image irradiates the charged photoconductor **21** with a light image irradiating device **24** to form an electrostatic latent image in the photoconductor **21**. The latent image is developed with a developing unit (not shown in FIG. 5) to form a toner image on the photoconductor **21**. The toner image is transferred onto a transfer paper (not shown) using a transfer charger **25**. After the toner image transferring process, the photoconductor **21** is cleaned by performing a pre-cleaning light irradiating operation using a pre-cleaning light irradiating device **26** and a cleaning brush **27**, and is then discharged with a discharging light source **28**. In the pre-cleaning light irradiating process, light irradiates the photoconductor **21** from the side of the substrate thereof. In this case, the substrate has to be light-transmissive.

The image forming apparatus of the present invention is not limited to the image forming units as shown in FIGS. 4 and 5. For example, in FIG. 5, the pre-cleaning light irradiating can be performed from the photoconductive layer side of the photoconductor **21**, and in addition, the light irradiation at the light image irradiating process and the discharging process can be performed from the substrate side of the photoconductor **21**. In addition, pre-transfer light irradiation, which is performed before the transferring of the toner image, and preliminary light irradiation of the image-wise light irradiation, which is performed before the image-wise light irradiation, and other light irradiation can also be performed.

The above-mentioned image forming units as shown in FIGS. 4 and 5 can be fixedly incorporated in image forming apparatuses such as copying machines, facsimile machines, printers and the like. Alternatively, the image forming units can be set in the image forming apparatuses as a process cartridge. The term "process cartridge" means a cartridge in which a charger, a light irradiating device, a developing device, a transfer device, a cleaning device, a discharging device and the like are set. Process cartridges having various shapes can be available in the present invention. A typical embodiment of the process cartridges of the present invention is shown in FIG. 6. FIG. 6 illustrates a compact process cartridge in which a charger **17**, a cleaning brush **18**, a light image irradiating device **19**, and a developing roller **20** are provided around a photoconductor **16**. The photoconductor **16** has a photoconductive layer which includes an organic pigment prepared by the method of the present invention and which is formed on an electroconductive substrate.

Having generally described this invention, further understanding can be obtained by reference to certain specific examples which are provided herein for the purpose of illustration only and are not intended to be limiting. In the descriptions in the following examples, the numbers represent weight ratios in parts, unless otherwise specified.

## EXAMPLES

At first, the method for synthesizing a titanyl phthalocyanine pigment which has a crystal form such that a maximum

diffraction peak is observed at a Bragg ( $2\theta$ ) angle of  $27.2^\circ \pm 0.2^\circ$  (so-called Y type titanyl phthalocyanine) when an X-ray of Cu—K  $\alpha$  having a wavelength of  $1.514 \text{ \AA}$  irradiates the crystal will be explained in detail.

### Example 1

In a container, 525 parts of phthalodinitrile and 4000 parts of 1-chloronaphthalene were contained and stirred. Under a nitrogen current, 190 parts of tetrachlorotitanium were dropped therein. After the addition of tetrachlorotitanium, the temperature of the mixture was gradually increased to  $200^\circ \text{ C}$ . The temperature of the mixture was maintained at a temperature range of from  $190$  to  $210^\circ \text{ C}$ . for 5 hours to react the compounds. After the reaction was terminated, the reaction product was cooled. When the temperature thereof cooled to  $130^\circ \text{ C}$ ., the reaction product was filtered. Then the filtered cake was washed with 1-chloronaphthalene until the cake colored blue. The cake was then washed with methanol several times, and further washed with hot water at  $80^\circ \text{ C}$ . several times. When the washed cake was dried, 422 parts of a rough titanylphthalocyanine pigment were obtained. Sixty (60) parts of the thus prepared rough titanylphthalocyanine pigment were added in 1000 parts of 96% sulfuric acid at a temperature of from  $3$  to  $5^\circ \text{ C}$ . while stirring, to dissolve the rough titanylphthalocyanine pigment. The solution was filtered, and the filtrate was dropped into 35 liters of iced water while stirring to deposit a crystal (titanylphthalocyanine pigment). The deposited crystal was filtered and then washed with water until the washing water became neutral (pH of 7.0). Thus, an aqueous paste of the titanylphthalocyanine pigment was prepared. One thousand and five hundred parts (1500) of 1,2-dichloroethane were added in the aqueous paste of the titanylphthalocyanine pigment, and the mixture was stirred for 2 hours at room temperature. Then 2500 parts of methanol were added therein, and the mixture was stirred and then filtered. The filtered cake was further washed with methanol. Thus, 98 parts of a wet cake of the pigment was prepared. When 50 parts of the wet cake were dried at  $65^\circ \text{ C}$ . in the atmosphere (760 mm Hg), 24 parts of a titanylphthalocyanine pigment were prepared. The solid content of the wet cake was 48% by weight.

### Example 2

When 48 parts of the wet cake prepared in Example 1 were dried at  $65^\circ \text{ C}$ . under a reduced atmospheric pressure, a phthalocyanine pigment of 24 parts were prepared. The solid content of the wet cake was 50% by weight.

### Example 3

The procedure for preparation of the wet cake of the titanylphthalocyanine pigment in Example 1 was repeated. The solid content of the wet cake was 59% by weight. The wet cake was subjected to vacuum drying at  $65^\circ \text{ C}$ . under a reduced atmospheric pressure of 5 mm Hg. Thus, a powder of the titanylphthalocyanine pigment was prepared.

### Example 4

The procedure for preparation of the wet cake of the titanylphthalocyanine pigment in Example 1 was repeated. The solid content was 68% by weight. The wet cake was subjected to vacuum drying at  $65^\circ \text{ C}$ . under a reduced atmospheric pressure of 5 mm Hg. Thus, a powder of the titanylphthalocyanine pigment was prepared.

### Comparative Example 1

Thirty (30) parts of the rough titanylphthalocyanine, which was prepared in Example 1 were treated with sulfuric

acid in the same way as performed in Example 1 to prepare an aqueous paste. Seven hundred and fifty (750) parts of 1,2-dichloroethane were added to the aqueous paste, and the mixture was stirred for 2 hours at room temperature. One thousand and two hundred fifty (1250) parts of methanol were added to the mixture, and the mixture was stirred and then filtered. The filtered cake was washed with methanol, and thereby 33.8 parts of a wet cake were prepared. The wet cake was dried at 65° C. under a reduced atmospheric pressure. Thus, a titanyl phthalocyanine pigment of 25 parts was obtained. The solid content of the wet cake was 74% by weight.

Each of the pigments obtained in Examples 1 to 4 and Comparative Example 1 was crushed with a marketed mixer to obtain a powder having a desired particle diameter. The mixing time was shown in Table 1.

TABLE 1

|                                | Mixing time                                                                                                                                                                   |
|--------------------------------|-------------------------------------------------------------------------------------------------------------------------------------------------------------------------------|
| Powder obtained in Ex. 1       | about 15 seconds                                                                                                                                                              |
| Powder obtained in Ex. 2       | about 10 seconds                                                                                                                                                              |
| Powder obtained in Ex. 3       | about 20 seconds                                                                                                                                                              |
| Powder obtained in Ex. 4       | about 25 seconds                                                                                                                                                              |
| Powder obtained in Comp. Ex. 1 | Powder having a uniform particle diameter could not be obtained even when the pigment was crushed for about 60 seconds. However, many large particles remained in the powder. |

X-ray irradiated the titanylphthalocyanine powders prepared in Examples 1 to 4 and Comparative Example 1 to obtain X-ray diffraction spectra. The conditions were as follows:

X-ray tube: copper  
Voltage: 40 kV  
Current: 20 mA  
Scanning speed: 1°/min  
scanning range: 3° to 4°  
Time constant: 2 seconds

The X-ray diffraction spectra of the powders obtained in Examples 1 to 4 were the same, and therefore the spectrum of the powder obtained in Example 2 is shown in FIG. 7 as a typical example. As can be understood from FIG. 7, the thus prepared titanylphthalocyanine pigment has a target crystal form such that a maximum peak of the X-ray diffraction spectrum is observed at a Bragg (2θ) angle of  $27.2^{\circ} \pm 0.2^{\circ}$ . Therefore the pigment has a desired crystal form (Y type).

The spectrum of the powder obtained in Comparative Example 1 is shown in FIG. 8. The spectrum has a crystal form such that a maximum peak of the X-ray diffraction spectrum is observed at an angle of  $26.3^{\circ} \pm 0.2^{\circ}$  other than the Bragg (2θ) angle of  $27.2^{\circ} \pm 0.2^{\circ}$ . Therefore the pigment has another crystal form (A type or β type). It is considered that the crystal change occurred during the crushing process because the processes of the synthesis process, sulfuric acid treatment process and crystal form changing process were performed in the same way. The reason of this crystal change is considered to be that the resultant pigment powder prepared in Comparative Example 1 had a high bulk density (i.e., the powder was firmly set), and therefore it takes a long time to crush the pigment powder, resulting in application of large stresses to the pigment during the crushing process.

Next, the method for manufacturing a photoconductor will be explained.

## Example 5

The following components were contained in a ball mill pot, which had a diameter of 90 mm and contained 600 g of PSZ balls having a particle diameter of 5 mm therein, and then dispersed for 2 hours at a rotation speed of 60 rpm to prepare a Dispersion 1.

Titanylphthalocyanine pigment powder prepared in Example 1 1.5

Polyvinyl butyral solution of methyl ethyl ketone 81 (polyvinyl butyral/methyl ethyl ketone=1/80)

## Example 6

The procedure for preparation of Dispersion 1 in Example 5 was repeated to prepare a Dispersion 2 except that the titanylphthalocyanine pigment powder prepared in Example 1 was replaced with 1.5 parts of the titanylphthalocyanine pigment powder prepared in Example 2.

## Example 7

The procedure for preparation of Dispersion 1 in Example 5 was repeated to prepare a Dispersion 3 except that the titanylphthalocyanine pigment powder prepared in Example 1 was replaced with 1.5 parts of the titanylphthalocyanine pigment powder prepared in Example 3.

## Example 8

The procedure for preparation of Dispersion 1 in Example 5 was repeated to prepare a Dispersion 4 except that the titanylphthalocyanine pigment powder prepared in Example 1 was replaced with 1.5 parts of the titanylphthalocyanine pigment powder prepared in Example 4.

## Comparative Example 2

The procedure for preparation of Dispersion 1 in Example 5 was repeated to prepare a Dispersion 5 except that the titanylphthalocyanine pigment powder prepared in Example 1 was replaced with 1.5 parts of the titanylphthalocyanine pigment powder prepared in Comparative Example 1.

## Comparative Example 3

The procedure for preparation of Dispersion 1 in Example 5 was repeated to prepare a Dispersion 6 except that the titanylphthalocyanine pigment powder prepared in Example 1 was replaced with 1.5 parts of the titanylphthalocyanine pigment powder prepared in Comparative Example 1 and the milling time was changed to 10 hours.

The particle size of the pigment particles in Dispersions 1 to 6 was measured with CAPA700 manufactured by HORIBA, LTD. In addition, Dispersions 1 to 6 were dried and X-ray irradiated the resultant powders under the same conditions mentioned above to obtain X-ray diffraction spectra of the powders.

The results are shown in Table 2.

TABLE 2

|                      | Average particle diameter (μm) | X-ray diffraction spectrum |
|----------------------|--------------------------------|----------------------------|
| Ex. 5 (Dispersion 1) | 0.37                           | Same as that in FIG. 7     |
| Ex. 6 (Dispersion 2) | 0.31                           | Same as that in FIG. 7     |
| Ex. 7 (Dispersion 3) | 0.36                           | Same as that in FIG. 7     |
| Ex. 8 (Dispersion 4) | 0.39                           | Same as that in FIG. 7     |

TABLE 2-continued

|                               | Average particle diameter ( $\mu\text{m}$ ) | X-ray diffraction spectrum                          |
|-------------------------------|---------------------------------------------|-----------------------------------------------------|
| Comp. Ex. 2<br>(Dispersion 5) | 0.78                                        | Same as that in FIG. 8                              |
| Comp. Ex. 3<br>(Dispersion 6) | 0.46                                        | The peak at the angle of $26.3^\circ$ became higher |

As can be understood from Table 2, the dispersion including a pigment prepared by the method of the present invention includes finely dispersed titanylphthalocyanine pigment particles, and the dispersed titanylphthalocyanine pigment maintains the desired crystal form.

### Example 9

On one side of an electrocasted nickel belt, the following undercoat layer coating liquid, charge generating layer coating liquid and charge transporting layer coating liquid were coated and dried one by one. Thus, a multi-layer type photoconductor was prepared.

| Formulation of undercoat layer coating liquid             |     |
|-----------------------------------------------------------|-----|
| Titanium dioxide powder                                   | 15  |
| Polyvinyl butyral                                         | 6   |
| 2-Butanone                                                | 150 |
| Formulation of charge generating layer coating liquid     |     |
| Dispersion 1                                              | 100 |
| Formulation of charge transporting layer coating liquid   |     |
| Polycarbonate                                             | 10  |
| Methylene chloride                                        | 80  |
| Charge transporting material having the following formula | 7   |

Charge transporting material having the following formula 7



Thus, a multi-layer type photoconductor of the present invention was prepared.

### Example 10

The procedure for preparation of the photoconductor in Example 9 was repeated except that Dispersion I in the charge generating layer coating liquid was replaced with Dispersion 2.

### Comparative Example 4

The procedure for preparation of the photoconductor in Example 9 was repeated except that Dispersion 1 in the charge generating layer coating liquid was replaced with Dispersion 6.

Each of the photoconductors prepared in Examples 9 and 10 and Comparative Example 4 was set in an image forming apparatus having the image forming unit as shown in FIG. 5, and 5000 images were continuously reproduced using a laser diode, which emitted light having a wavelength of 780 nm, as the light source of the light image irradiating device. Light image irradiated the photoconductor via a polygon mirror. In addition, the pre-cleaning light irradiation was not performed. Further, a probe of a surface potential meter was set in the apparatus to measure the initial surface potentials of two areas of each photoconductor, one of which was exposed to light and the other of which was not exposed to light. Further, the surface potentials of the two areas were also measured at  $5000^{\text{th}}$  image forming operation.

The results are shown in Table 3.

TABLE 3

|             | Initial surface potential (V) | Surface potential at the $5000^{\text{th}}$ image forming operation (V) |                                 |
|-------------|-------------------------------|-------------------------------------------------------------------------|---------------------------------|
|             |                               | Area which was not exposed to light                                     | Area which was exposed to light |
| Ex. 9       | -851                          | -120                                                                    | -838                            |
| Ex. 10      | -853                          | -110                                                                    | -847                            |
| Comp. Ex. 4 | -903                          | -230                                                                    | -888                            |

As can be understood from Table 3, the photoconductor of the present invention has good charge properties and can maintain the charge properties even when repeatedly used for a long time.

### Example 11

The surface of an aluminum cylinder was subjected to an anodic oxidation treatment and then was sealed. The following charge generating layer coating liquid and charge transporting layer coating liquid were then coated and dried one by one, to form a charge generating layer of  $0.2\ \mu\text{m}$  thick and a charge transporting layer of  $20\ \mu\text{m}$  thick thereon. Thus, a photoconductor of the present invention was prepared.

| Formulation of charge generating layer coating liquid     |     |
|-----------------------------------------------------------|-----|
| Dispersion 1                                              | 100 |
| Formulation of charge transporting layer coating liquid   |     |
| Polycarbonate                                             | 10  |
| Methylene chloride                                        | 80  |
| Charge transporting material having the following formula | 8   |



Thus, a multi-layer type photoconductor of the present invention was prepared.

#### Example 12

The procedure for preparation of the photoconductor in Example 11 was repeated except that the charge generating layer coating liquid was replaced with 100 parts of Dispersion 3. Thus a photoconductor of the present invention was prepared.

#### Example 13

The procedure for preparation of the photoconductor in Example 11 was repeated except that the charge generating layer coating liquid was replaced with 100 parts of Dispersion 4. Thus a photoconductor of the present invention was prepared.

#### Comparative Example 5

The procedure for preparation of the photoconductor in Example 11 was repeated except that the charge generating

polygon mirror. The image qualities of the initial image and the 3000th image were visually observed. The results are shown in Table 4.

TABLE 4

|             | Initial image qualities                                     | Image qualities of 3000 <sup>th</sup> image.                                             |
|-------------|-------------------------------------------------------------|------------------------------------------------------------------------------------------|
| Ex. 11      | good                                                        | good                                                                                     |
| Ex. 12      | good                                                        | good                                                                                     |
| Ex. 13      | good                                                        | good                                                                                     |
| Comp. Ex. 5 | Image defects occurred which were caused by coating defects | Image defects occurred which were caused by coating defects, and image density decreased |

As can be understood from Table 4, the photoconductor of the present invention can maintain good image qualities even when used for a long time.

#### Example 14

The procedure for preparation of the photoconductor in Example 9 was repeated except that the electrocasted nickel belt substrate was replaced with an aluminum cylinder substrate.

Thus a photoconductor of the present invention was prepared.

#### Example 15

The procedure for preparation of the photoconductor in Example 14 was repeated except that the formulation of the charge transporting layer coating liquid was changed to the following formulation.

##### Formulation of charge transporting layer coating liquid

Methylene chloride 100

High molecular weight charge transporting material having the following formula 10



layer coating liquid was replaced with 100 parts of Dispersion 5. Thus a comparative photoconductor was prepared.

Each of the photoconductors prepared in Examples 11 to 13 and Comparative Example 5 was set in an electrophotographic process cartridge as shown in FIG. 6, and the cartridge was set in an image forming apparatus. Three thousand (3000) images were continuously reproduced using a laser diode, which emitted light having a wavelength of 780 nm, as the light source of the light image irradiating device. Light image irradiated the photoconductor via a

#### Example 16

The procedure for preparation of the photoconductor in Example 14 was repeated except that the formulation of the charge transporting layer coating liquid was changed to the following formulation.

##### Formulation of charge transporting layer coating liquid

Methylene chloride 100

High molecular weight charge transporting material having the following formula 10



Each of the photoconductors prepared in Examples 14 to 16 was set in an electrophotographic image forming apparatus as shown in FIG. 4. Ten thousand (10000) images were continuously reproduced using a laser diode, which emitted light having a wavelength of 780 nm, as the light source of the light image irradiating device. Light image irradiated the photoconductor via a polygon mirror. The image qualities of the initial image and the 10000th image were visually observed. In addition, the thickness of the photoconductive layer of each photoconductor was measured before and after the running test to determine a decrease of the thickness. The results are shown in Table 5.

TABLE 5

|        | Initial image qualities | Image qualities of 10000 <sup>th</sup> image                   | Decrease of photoconductive layer (μm) |
|--------|-------------------------|----------------------------------------------------------------|----------------------------------------|
| Ex. 14 | good                    | Slight black stream occurred, but it is on an acceptable level | 2.8                                    |
| Ex. 15 | good                    | good                                                           | 1.0                                    |
| Ex. 16 | good                    | good                                                           | 1.1                                    |

As can be understood from Table 5, the photoconductors of Examples 15 and 16 of the present invention have good abrasion resistance.

As mentioned above, according to the present invention, a method is provided for effectively preparing an organic pigment useful for an electrophotographic photoconductor. By using this method, a coating liquid in which an organic pigment having a fine particle diameter is dispersed without changing its crystal form can be prepared. The coating liquid is useful for forming photoconductive layer, and the resultant photoconductive layer has good charge properties and few coating defects. Therefore, a photoconductor having high sensitivity, stable charge properties and good abrasion resistance can be provided. In addition, an image forming apparatus and process cartridge which includes the photoconductor of the present invention and which can produce images having good image qualities even when repeatedly used for a long time can also be provided.

Additional modifications and variations of the present invention are possible in light of the above teachings. It is therefore to be understood that within the scope of the appended claims the invention may be practiced other than as specifically described herein.

This document claims priority and contains subject matter related to Japanese Patent Application No. 10-225177, filed on Jul. 27, 1998, the entire contents of which are herein incorporated by reference.

What is claimed is:

1. An organic pigment dispersion useful for forming an electrophotographic photoconductor which comprises at

15 least an organic pigment and a solvent, wherein the organic pigment is prepared by a method in which an organic pigment wet cake which includes at least the organic pigment and a solvent which may be chemically different from or the same as said first-mentioned solvent is provided, and then dried by being heated at a temperature higher than room temperature to prepare a powder of the organic pigment, and wherein the organic pigment is present in the organic pigment wet cake in an amount of not greater than about 70% by weight at the beginning of heating.

20 2. The organic pigment dispersion according to claim 1, wherein the organic pigment comprises a titanyl phthalocyanine compound having an X-ray diffraction spectrum such that a maximum peak is observed at a Bragg (2θ) angle of 27.2°±0.2° when an X-ray of Cu—K α having a wavelength of 1.514 Å irradiates the titanyl phthalocyanine compound.

25 3. An electrophotographic photoconductor comprising an electroconductive substrate and a photoconductive layer which is formed overlying the electroconductive substrate and which comprises an organic pigment, wherein the organic pigment is prepared by a method in which an organic pigment wet cake which includes at least the organic pigment and a solvent is provided, and then dried by being heated at a temperature higher than room temperature to prepare a powder of the organic pigment, and wherein the organic pigment is present in the organic pigment wet cake in an amount of not greater than about 70% by weight at the beginning of heating.

30 4. The electrophotographic photoconductor according to claim 3, wherein the photoconductive layer comprises a charge generating layer and a charge transporting layer.

35 5. The electrophotographic photoconductor according to claim 4, wherein the charge transporting layer comprises a polycarbonate resin having a triarylamine structure in at least one of a main chain and a side chain thereof.

40 6. An image forming method comprising the steps of: providing an electrophotographic photoconductor comprising an electroconductive substrate and a photoconductive layer which is formed overlying the electroconductive substrate and which comprises an organic pigment,

45 55 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575

which an organic pigment wet cake which includes at least the organic pigment and a solvent is provided, and then dried by being heated at a temperature higher than room temperature to prepare a powder of the organic pigment, and wherein the organic pigment is present in the organic pigment wet cake in an amount of not greater than about 70% by weight at the beginning of heating.

7. An image forming apparatus comprising:

- an electrophotographic photoconductor comprising an electroconductive substrate and a photoconductive layer which is formed overlying the electroconductive substrate and which comprises an organic pigment,
- a charging device which charges the electrophotographic photoconductor,
- a light image irradiating device which irradiates the charged electrophotographic photoconductor with imagewise light to form an electrostatic latent image thereon,
- a developing device which develops the electrostatic latent image with a toner to form a toner image on the electrophotographic photoconductor,
- a transferring device which transfers the toner image onto a receiving material,
- a cleaning device which cleans a surface of the electrophotographic photoconductor, and

5

10

15

20

25

a discharging device which discharges the electrophotographic photoconductor, wherein the organic pigment is prepared by a method in which an organic pigment wet cake which includes at least the organic pigment and a solvent is provided, and then dried by being heated at a temperature higher than room temperature to prepare a powder of the organic pigment, and wherein the organic pigment is present in the organic pigment wet cake in an amount of not greater than about 70% by weight at the beginning of heating.

8. An image forming process cartridge comprising:

- an electrophotographic photoconductor comprising an electroconductive substrate and a photoconductive layer which is formed overlying the electroconductive substrate and which comprises an organic pigment,

wherein the organic pigment is prepared by a method in which an organic pigment wet cake which includes at least the organic pigment and a solvent is provided, and then dried by being heated at a temperature higher than room temperature to prepare a powder of the organic pigment, and wherein the organic pigment is present in the organic pigment wet cake in an amount of not greater than about 70% by weight at the beginning of heating.

\* \* \* \* \*